

July 31, 1962

C. J. MALM ET AL

3,047,391

METHOD OF COATING PARTIALLY ACETYLATED PAPER WITH PLASTICIZED  
CELLULOSE ESTER AND RESULTING PAPER COATED  
WITH A PHOTOGRAPHIC EMULSION

Filed Jan. 12, 1959

**SILVERHALIDE EMULSION LAYER**

**PAPER BASE OF PARTIALLY ACETYLATED  
CELLULOSE FIBERS IMPREGNATED WITH  
LOWER FATTY ACID ESTER OF CELLULOSE  
AND PLASTICIZER**

**Carl J. Malm  
Lloyd E. Herdle  
Gerald C. Gandy**  
INVENTORS

BY *R. Frank Smith*  
*Scranton C. Van Horsten*  
ATTORNEYS

1

3,047,391

## METHOD OF COATING PARTIALLY ACETYLATED PAPER WITH PLASTICIZED CELLULOSE ESTER AND RESULTING PAPER COATED WITH A PHOTOGRAPHIC EMULSION

Carl J. Malm, Lloyd E. Herdle, and Gerald C. Gandy, Rochester, N.Y., assignors to Eastman Kodak Company, Rochester, N.Y., a corporation of New Jersey

Filed Jan. 12, 1959, Ser. No. 786,043

7 Claims. (Cl. 96—85)

This invention relates to a method of improving the physical properties of partially acetylated paper.

A simplified flow diagram of the method is as follows:



Paper is ordinarily prepared from cellulose fibers such as wood pulp by applying a slurry of the fibers to the wire of a papermaking machine from which the thus formed paper is led eventually to calender rolls to impart a smooth, even finish thereto. To improve the characteristics of such paper, sizing agents may be applied either to the paper or to the fibers prior to their formation into paper. However, paper made from partially acetylated cellulose fibers often exhibits considerable resistance to sizing operations.

One object of our invention is to provide a partially acetylated paper useful for photographic purposes, the wet strength and fold values of which are comparable with, or better than, those of papers normally used as a photographic paper base. Another object of our invention is to provide a paper which is highly resistant to the effects of moisture and to change in dimensional stability. Other objects of our invention will appear herein.

We have found that paper having highly desirable characteristics may be obtained if paper is formed from pulp which has been partially acetylated so as to impart an acetyl content of 15-30% and that paper is treated with an alcohol solution of a cellulose ester and a plasticizer. The sheets of paper of this type have good wet strength and fold characteristics and the mullen and other properties are greatly improved. The cellulose fiber employed in making the paper is wood pulp which has been partially acetylated such as by some method described in the prior art or by the method described in U.S. application Ser. No. 786,045 of Herdle and Gandy, now abandoned, filed of even date, or in U.S. application Ser. No. 786,042 of Malm and Blanchard, now abandoned, filed of even date. Procedures for partially acetylating cellulose fiber are described in British Patent No. 367,312, U.S. application Ser. Nos. 469,624 and 469,846 of Richter et al., filed November 18, 1954, both now abandoned, and in an article entitled "Effect of Acetylation on Water-Binding Properties of Cellulose," in Industrial and Engineering Chemistry, volume 35, pages 1206-1210, November 1943. After the cellulose fibers have been partially acetylated they are formed into a sheet by any conventional papermaking procedure such as in a handsheet mold or on the wire of a paper machine. The paper thus prepared after

2

drying is treated with an alcohol solution of cellulose ester and plasticizer and after subjecting to pressure such as squeeze rolls and evaporation of the alcohol the paper is subjected to heat and pressure to give a smooth finish to the paper. The prevent the paper from losing its opacity, a pigment such as titanium dioxide can be incorporated in the solution as described and claimed in U.S. application Ser. No. 786,431 of Malm and Gandy, filed of even date.

10 The accompanying drawing represents in symbolic form, photographic paper having a paper base in accordance with the invention.

Many processes for partially acetylating wood pulp fibers actually decrease their strength and, consequently, 15 paper prepared therefrom is less strong than that prepared from fibers which had not been acetylated. However, whether or not partial acetylation has decreased the strength of the pulp fibers to any appreciable extent the treatment of paper sheets prepared therefrom with an 20 aliphatic alcohol solution of a cellulose ester and a plasticizer for the cellulose compound has a beneficial effect upon the properties of the paper.

The alcohols which are of value in this connection are 25 those of 1-4 carbon atoms such as butyl, isobutyl, propyl, isopropyl, ethyl and methyl. These alcohols have substantially no swelling effect on the partially acetylated fibers which is of particular advantage as the paper fibers take up only a minimum of the alcohol solution. For instance, 30 with some types of solvents as much as 4 parts of solution will be retained by the paper, whereas the retention of the alcohol solution by the fiber can be held to less than 1 part of solution per part of paper.

The treatment of paper with alcohol solution of cellulose ester and plasticizer gives a paper through which water 35 vapor will readily pass and also prevents much of the cockle effect upon subsequent rewetting and drying of the paper. The treatment described gives a uniform distribution of the cellulose ester and plasticizer therefor throughout the paper. The cellulose ester composition readily adheres to the fibers because of its affinity for partially acetylated material. The cellulose esters whose alcohol 40 solutions are employed are preferably the butyrate and propionates of cellulose. A certain amount of acetyl will be tolerated but there should be present sufficient propionyl or butyryl that the cellulose ester employed is readily soluble in hot alcohol. If the alcohol solution is only liquid at an elevated temperature, it is desirable to first heat the paper prior to subjecting it to treatment therewith. In the case of alcohols which are not readily compatible with 45 water, such as the butyl alcohols, heating of the paper initially is desirable to remove moisture therefrom. For instance, the paper prior to treatment may be subjected to a temperature of at least 120° F., the upper temperature limit being governed in part by that which will act derogatorily upon the paper. The plasticizer used may be any 50 plasticizer for the cellulose ester, it being employed in considerable proportion such as 20 to 75% of the cellulose ester-plasticizer mixture. Some plasticizers which are useful in this connection are dibutyl phthalate, dibutyl 55 sebacate, diethyl phthalate, dibutyl adipate, and the like.

The partially acetylated paper treated in accordance with 60 our invention is one which has been prepared from wood pulp fibers having an acetyl content of 15-25%. If the partially esterified fibers used have other acyl groups there- 65 in such as propionyl or butyryl the fibers employed should have an apparent acetyl content of 15-25%.

Treatment in accordance with our invention is conveniently carried out by immersing the paper in the alcohol 70 solution of cellulose ester and plasticizer such as by running it through a bath therof. This procedure can be very conveniently carried out in a continuous manner wherein a roll of paper is continuously unwound, heated

and passed into a bath of the alcohol solution and the paper is continuously withdrawn through squeeze rolls, the alcohol evaporated off and the paper passed over hot calender rolls thereby subjecting it to heat and pressure to give a smooth finish which is stable to water wetting and redrying. As the paper is not swollen, the amount of solution left in the paper is less than 1 part per part of paper. Upon evaporation of the alcohol the amount of cellulose ester and plasticizer which is retained in paper of usual thickness and absorbency is ordinarily less than  $\frac{1}{4}$  part per part of paper and preferably on the order of  $\frac{1}{10}$  part per part of paper.

In the case of the use of ethyl alcohol the pick up of the alcohol solution by the paper is greater than with the higher alcohols such as those of 3 or 4 carbon atoms. The solution employed ordinarily contains approximately 25% of cellulose ester and plasticizer dissolved in the alcohol. However, this concentration is optional as the solution can be considerably more dilute and will give interesting results in that the physical properties of the paper will be markedly improved. On the other hand, the amounts of cellulose ester and plasticizer used can be considerably more.

The following example illustrates our invention.

#### Example 1

Paper having a weight of 20 pounds per 1000 sq. ft. was made from a bleached kraft pulp which had been acetylated to an acetyl content of approximately 20%. This paper was passed through a solution consisting of 75% of n-butyl alcohol, 12.5% of half-second viscosity cellulose acetate butyrate (butyryl 35-39%, acetyl 12-15%) and 12.5% of dibutyl phthalate. The paper was passed through squeeze rolls to remove liquid therefrom leaving approximately  $\frac{1}{2}$  part of solution per part (by weight) of pulp. The alcohol in the paper sheet was evaporated therefrom by a current of warm dry air and the sheet obtained was supercalendered at 140° F. using 4 nips. This procedure was repeated on a paper which had been prepared as described but in which 1% of melamine formaldehyde resin had been incorporated in the paper stock prior to its manufacture on the wire of the paper machine. The following table lists the difference in physical properties between the paper in each case which had not been treated with an alcohol solution of cellulose ester and plasticizer and a paper which had been so treated. The paper in which the melamine formaldehyde resin had been incorporated is designated "wet strength paper."

5

10

15

20

25

30

35

40

45

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

The paper prepared in accordance with our invention is useful for preparing photographic paper by applying a silver halide emulsion layer thereon particularly after the paper had first been coated with a baryta layer as is well known in the art. It is desirable in the case of photographic use that the paper be prepared from a bleached pulp. However, our invention also contemplates the use of the treatment described upon paper made from unbleached pulp, which paper is useful for wrapping materials for electrical insulation or in any case where moisture absorption, resistance to swelling or dimensional change by moisture is important.

We claim:

1. A method of preparing paper resistant to the effect of moisture which comprises impregnating paper essentially consisting of partially acylated cellulose fibers with a solution in lower alcohol of a mixture of lower fatty acid ester of cellulose and a plasticizer therefor, in such manner as to leave less than 1 part of solution per part of paper, evaporating off the alcohol therefrom and subjecting to heat and pressure to impart a smooth finish to the paper.

2. A method of preparing paper resistant to the effect of moisture which comprises impregnating paper essentially consisting of partially acylated cellulose fibers with a solution in a lower alcohol of a mixture of lower fatty acid ester of cellulose and a plasticizer therefor, in such manner as to leave less than 1 part of solution per part of paper, evaporating off the alcohol therefrom and subjecting to heat and pressure to impart a smooth finish to the paper.

3. A method of preparing paper resistant to the effect of moisture which comprises impregnating paper essentially consisting of partially acylated cellulose fibers with a solution in a lower alcohol of a propionic acid ester of cellulose and a plasticizer therefor, in such manner as to leave less than 1 part of solution per part of paper, evaporating off the alcohol therefrom and subjecting to heat and pressure to impart a smooth finish to the paper.

4. A method of preparing paper resistant to the effect of moisture which comprises impregnating paper essentially consisting of partially acylated cellulose fibers

10

20

30

35

40

with a solution in a lower alcohol of a butyric acid ester of cellulose and a plasticizer therefor, in such manner as to leave less than 1 part of solution per part of paper, evaporating off the alcohol therefrom and subjecting to heat and pressure to impart a smooth finish to the paper.

5. A method of preparing paper resistant to the effect of moisture which comprises impregnating paper essentially consisting of partially acetylated cellulose fibers with a solution in a butyl alcohol of a mixture of a lower fatty acid ester of cellulose and a plasticizer therefor, in such manner as to leave less than 1 part of solution per part of paper, evaporating off the alcohol therefrom and subjecting to heat and pressure to impart a smooth finish to the paper.

15. 6. A method of preparing paper resistant to the effect of moisture which comprises impregnating paper essentially consisting of partially acetylated bleached kraft pulp with a solution in butyl alcohol of a butyric acid ester of cellulose and dibutyl phthalate as the plasticizer for the cellulose ester, passing the paper through squeeze rolls to remove liquid therefrom, thereby leaving approximately  $\frac{1}{2}$  part of solution per part of paper, evaporating off the alcohol therefrom and subjecting to heat and pressure to impart a smooth finish to the paper.

25. 7. Photographic paper comprising a paper base essentially consisting of partially acylated cellulose fibers which have been impregnated with a lower alcohol solution of a lower fatty acid ester of cellulose and a plasticizer from which paper the alcohol had been evaporated off and heat and pressure had been applied thereto and a photographic silver halide emulsion layer.

References Cited in the file of this patent

UNITED STATES PATENTS

|           |                  |                |
|-----------|------------------|----------------|
| 2,103,640 | Richter          | Dec. 28, 1937  |
| 2,186,957 | Collings et al.  | Jan. 16, 1940  |
| 2,227,494 | Gold             | Jan. 7, 1941   |
| 2,287,348 | Hayden           | June 23, 1942  |
| 2,351,174 | Whitehead        | June 13, 1944  |
| 2,357,962 | Leemann et al.   | Sept. 12, 1944 |
| 2,814,617 | Hagenbuch et al. | Nov. 26, 1957  |
| 2,955,958 | Brown            | Oct. 11, 1960  |